

# United States Patent Office

2,971,915

Patented Feb. 14, 1961

1

2,971,915

## LUBRICATING OIL COMPOSITIONS

Victor N. Borsoff and George M. Calhoun, Berkeley, Calif., assignors to Shell Oil Company, a corporation of Delaware

No Drawing. Filed Feb. 11, 1957, Ser. No. 639,237

18 Claims. (Cl. 252—56)

This invention relates to lubricants, particularly those suitable for lubrication under severe operating conditions, such as under extreme high speed and at high temperatures.

It is well known that the high pressure occurring in certain types of gears and bearings may cause rupture of lubricant films with consequent damage to the machinery. It has been shown that various base lubricants can be improved in their protective properties for rubbing surfaces by the addition of certain substances, so-called extreme pressure agents, so that excessive wear, scuffing and seizure which normally follow a break in the film lubricant, can be minimized or prevented.

It is known that certain compounds of metal-reactive elements, such as certain compounds of chlorine, sulfur and phosphorus, as well as certain other compounds, such as some compounds of lead, impart extreme pressure properties to various lubricants. Notable among the substances heretofore used are the lead soaps, phosphoric acid esters, free or bound sulfur and certain chlorinated organic compounds. A principal objection to many of these extreme pressure agents is their generally high reactivity with the metallic surface, causing etching, corrosion and discoloration of the metal surface. Another objection to chemically reactive extreme pressure agents is that they alter the original chemical nature of the contacting surface, which under certain conditions is undesirable. Additionally, because of the activity of agents of this type, they usually are depleted rapidly resulting in only a temporary solution to the problem of extreme pressure lubrication.

It has now been discovered that improved extreme pressure lubricants are provided by a suitable lubricating oil containing certain marginally oil-soluble aliphatic dicarboxylic acids. The aliphatic dicarboxylic acids have the formula  $\text{HOOC}_n\text{H}_{2n-m}\text{R}_m\text{COOH}$ , wherein R is an alkyl radical of from 1 to 4 carbon atoms, n is an integer of from 3 to 6, m is an integer of from 1 to 6 inclusive, and the total number of carbon atoms in all R's is from 1 to 6. The dibasic acids are  $\text{C}_{1-4}$ -alkyl substituted glutaric, adipic, pimelic or suberic acids, wherein the two acid groups are separated by a chain of from 3 to 6 carbon atoms. One or more of the connecting carbon atoms is substituted with alkyl, preferably methyl, radicals to a total of from 1 to 6 carbon atoms in all alkyl radicals in a given molecule, preferably no more than three.

The acid groups must be separated by a chain of three to six carbon atoms to provide the superior extreme pressure properties and in addition the separating alkylene radical  $-\text{C}_n(\text{H}_{2n-m}\text{R}_m)-$  must contain at least one side-chain alkyl radical (R) in order to provide the minimum required oil solubility while not unduly adversely affecting the extreme pressure properties of the dibasic acid. Dibasic acids in which the acid groups are separated by less than three carbon atoms, such as succinic acid, or by more than six carbon atoms, such as sebastic acid, have been found to be poor extreme pressure agents,

2

even when one or more of the connecting carbon atoms is substituted with an alkyl radical of from 1 to 6 or more carbon atoms.

The useful dibasic acids in general are marginally oil-soluble. However, they should be soluble in oil to the extent of at least about 0.5% by weight, better at least 1% by weight, but not over about 10% by weight and preferably not over about 5% by weight. The solubility of the acids in the oil can be increased by providing oil-soluble branched-chain aliphatic alcohols, in the oil as a solubilizing agent. These alcohols effectively solubilize the dibasic acids of lower oil-solubility while the acids retain their extreme pressure properties in the oil.

More specifically, the dibasic acids are represented by such substances as the 2-, 2,2-, 2,3-, 3-, 3,3-, 4-, 4,4-, 2,4-, 2,5-, 2,3,4-, 2,3,5-, mono, di, and tri, methyl or ethyl or 2-, or 3-, monobutyl glutaric, adipic, pimelic or suberic acids. Preferred acids are 2-methyl glutaric acid, 2-methyl adipic acid, 2-methyl pimelic acid, 2-methyl suberic acid, 3-methyl glutaric acid, 3-methyl adipic acid, 3-methyl pimelic acid, 3-methyl suberic acid, 2,2-dimethyl glutaric acid, 2,2-dimethyl adipic acid, 2,3-dimethyl glutaric acid, 2,3-dimethyl adipic acid, 3,3-dimethyl adipic acid, 2,4-dimethyl adipic acid, 2,2,4-trimethyl adipic acid, 2,3,4-trimethyl adipic acid, 2,2,4-trimethyl suberic acid, 3-ethyl glutaric acid, 2-methyl, 3-ethyl adipic acid, 2-methyl-4-butyl suberic acid and mixtures thereof.

These extreme pressure agents are miscible in mineral lubricating oils at room or storage temperatures up to about 2% by weight. When it is desired to incorporate an amount of dibasic acid in the oil in excess of its oil-solubility at room temperature, a branched-chain alkanol is useful. These alkanols effectively solubilize the dibasic acids so that amounts of as high as 10% by weight, based on the total oil compositions, can be dispersed in the oil.

Particularly useful alkanols for the purpose of solubilizing the dibasic acids, without interfering with their extreme pressure activity, are the so-called "Oxo" alcohols derived from branched-chain olefins, such as polymers of lower alkenes of 3 to 5 carbon atoms, and copolymers of mixtures of such alkenes by catalyzed reaction with carbon monoxide and hydrogen in accordance with the conditions of the "Oxo" process, as is well known in the art. The composition of a typical  $\text{C}_8$ -Oxo-alcohol mixture derived from a mixture of  $\text{C}_7$ -olefins, produced by polymerization of a typical refinery cracked gas fraction of  $\text{C}_5$ — $\text{C}_4$  hydrocarbons, is given in Table I.

TABLE I

|    | Alcohol                  | Percent, wt. |
|----|--------------------------|--------------|
| 55 | 3,5-dimethyl hexanol     | 29           |
|    | 4,5-dimethyl hexanol     | 25           |
|    | 3,4-dimethyl hexanol     | 17           |
|    | 5-methyl heptanol        | 16           |
|    | 3-methyl heptanol        | 2.3          |
|    | 5-ethyl hexanol          | 1.4          |
|    | 5,5-dimethyl hexanol     | 4.3          |
| 60 | $\alpha$ -alkyl alkanols | 5.0          |
|    | Others                   |              |

Other examples of suitable alkanols include 6-methyl-1-heptanol, 2-n-propyl-1-pentanol, 3-n-propyl-1-hexanol, 2,2-dimethyl-1-octanol, 10,10-dimethyl-1-undecanol, 3-isopropyl-1-heptanol and mixtures thereof.

The lubricating oils used in compositions of this invention can be a variety of synthetic or natural hydrocarbon oils having a viscosity range of from 5W SUS at 100° F. to 250 SUS at 210° F. (SAE viscosity number 70 ranging from SAE 50 to SAE 90). The natural hydrocarbon oils can be obtained from paraffinic, naphthenic, asphaltic or mixed base crudes, and/or mixtures thereof.

Synthetic oils include polymerized olefins, alkylated aromatics, isomerized waxes, copolymers of alkylene glycols and alkylene oxide (Ucon fluids) which are described in U.S. Patents 2,425,755, 2,425,845 and 2,774,733 such as Ucon 50HB170, Ucon 50HB660 or Ucon LB550X and which are copolymers of ethylene and 1,2-propylene oxides the mono and diols as well as their ether derivatives; organic esters of an aliphatic dibasic acid such as di-2-ethyl hexyl sebacate or di-2-ethyl hexyl adipate and the like. The hydrocarbon oils may be blended with fixed oils such as castor oil, lard oil and the like and/or synthetic oils as mentioned or silicone polymers and the like. Typical oils of this type are petroleum motor oils (A) which is paraffinic in character and (B) which is naphthenic in character having the following properties:

|                               | (A)<br>(SAE 10W) | (B)<br>(SAE 30) |
|-------------------------------|------------------|-----------------|
| Pour Point, °F.....           | -10              | -5              |
| Flash, °F.....                | 390              | 415             |
| Viscosity, SUS at 210° F..... | 44               | 58              |
| Viscosity Index.....          | 90               | 80              |

Other suitable oils are the gas turbine lube oils having the following properties:

| Grade.....                    | 1010 | 1065 |
|-------------------------------|------|------|
| Flash, COC, °F.....           | 300  | 465  |
| Pour, °F.....                 | -10  | 0    |
| Viscosity, SUS at 100° F..... | 59.4 | 530  |
| Neutral Number.....           | 0.02 | 0.01 |
| Ash.....                      | None | None |

Compositions A through O are representative of the invention wherein the base oils are identified hereinabove:

| Composition A:               | Percent wt. |
|------------------------------|-------------|
| 3-methyl glutaric acid ..... | 2           |
| 1010 mineral oil .....       | Balance     |

| Composition B:                   | Percent wt. |
|----------------------------------|-------------|
| 3,3-dimethyl glutaric acid ..... | 2           |
| 1010 mineral oil .....           | Balance     |

| Composition C:                   | Percent wt. |
|----------------------------------|-------------|
| 2,2-dimethyl glutaric acid ..... | 2           |
| 1010 mineral oil .....           | Balance     |

| Composition D:             | Percent wt. |
|----------------------------|-------------|
| 3-methyl adipic acid ..... | 2           |
| 1010 mineral oil .....     | Balance     |

| Composition E:                 | Percent wt. |
|--------------------------------|-------------|
| 2,4-dimethyl adipic acid ..... | 2           |
| 1010 mineral oil .....         | Balance     |

| Composition F:                    | Percent wt. |
|-----------------------------------|-------------|
| 2,2,4-trimethyl adipic acid ..... | 2           |
| 1010 mineral oil .....            | Balance     |

| Composition G:                    | Percent wt. |
|-----------------------------------|-------------|
| 2-methyl pimelic acid .....       | 2           |
| C <sub>10</sub> Oxo alcohol ..... | 3           |
| 1010 mineral oil .....            | Balance     |

| Composition H:              | Percent wt. |
|-----------------------------|-------------|
| 2-methyl suberic acid ..... | 2           |
| 1010 mineral oil .....      | Balance     |

| Composition I:                    | Percent wt. |
|-----------------------------------|-------------|
| 3-methyl glutaric acid .....      | 3           |
| C <sub>10</sub> Oxo alcohol ..... | 3           |
| 1010 mineral oil .....            | Balance     |

| Composition J:                          | Percent wt. |
|-----------------------------------------|-------------|
| 3-methyl glutaric acid .....            | 3           |
| C <sub>10</sub> Oxo alcohol .....       | 3           |
| 2,6-di-tert butyl-4-methyl phenol ..... | 0.1         |
| 1010 mineral oil .....                  | Balance     |

|                                   | Percent wt. |
|-----------------------------------|-------------|
| Composition K:                    |             |
| 3-methyl adipic acid .....        | 2           |
| Mineral oil (B) .....             | Balance     |
| Composition L:                    |             |
| 3-ethyl adipic acid .....         | 2           |
| C <sub>10</sub> Oxo alcohol ..... | 3           |
| Mineral oil (B) .....             | Balance     |
| Composition M:                    |             |
| 2,3-dimethyl adipic acid .....    | 2           |
| Ucon 50HB660 .....                | Balance     |
| Composition N:                    |             |
| 2,3-dimethyl adipic acid .....    | 2           |
| Ucon LB-550X .....                | Balance     |
| Composition O:                    |             |
| 2,3-dimethyl adipic acid .....    | 2           |
| Di-2-ethyl hexyl sebacate .....   | Balance     |

Compositions of this invention were evaluated for their extreme pressure properties on a spur-gear machine, which essentially consists of two geometrically similar pairs of gears connected by two parallel shafts. The gear pairs are placed in separate gear boxes, which also contain the supporting ball bearings. One of the shafts consists of two sections connected by a coupling. Loading is accomplished by locking one side of the coupling and applying torque to the other. The conditions of the test were:

Speed ..... r.p.m. 3200

Oil temperature ..... °F. 100

Oil flow-rate ..... cc./scc. 10

Load in increments 5 min. at each setting.

Results of the evaluations are given in Table II. For purpose of comparison, the results obtained from the use of the base oil alone, and with other dicarboxylic acids, are also given in Table II.

TABLE II  
Spur gear machine test results

| Composition:                                                    | Load (lb./in.) |
|-----------------------------------------------------------------|----------------|
| A.....                                                          | 9,900          |
| B.....                                                          | 7,100          |
| C.....                                                          | 7,100          |
| D.....                                                          | 10,400         |
| E.....                                                          | 12,500+        |
| F.....                                                          | 9,200          |
| G.....                                                          | 12,700         |
| H.....                                                          | 12,500         |
| I.....                                                          | 9,900          |
| J.....                                                          | 10,000         |
| K.....                                                          | 10,000         |
| L.....                                                          | 10,000         |
| M.....                                                          | 12,000         |
| N.....                                                          | 10,600         |
| O.....                                                          | 8,500          |
| 1010 mineral oil +2% succinic acid.....                         | 1,400          |
| 1010 mineral oil +2% C <sub>16</sub> alkenyl succinic acid..... | 2,800          |
| SAE 10 mineral oil +2% malonic acid.....                        | 1,800          |
| 1010 mineral oil +2% 3-hexadecyl adipic acid.....               | 1,400          |
| SAE 10W mineral oil.....                                        | 600            |
| 1010 mineral oil.....                                           | 600            |

Thus, the data show the outstanding enhancement of the load-carrying ability of the oil effected by the dicarboxylic acids of the invention, as represented by those of Compositions A through O. On the other hand, malonic acid and succinic acid in which the two carboxylic acid groups are separated by only one and two carbon atoms, respectively, and C<sub>16</sub>-alkenyl succinic acid in which oil-solubility is obtained by the C<sub>16</sub>-hydrocarbon radical effected only a slight improvement. Also whereas 3-methyl adipic acid (Composition D) increased the load capacity from 600 to 10,000 pounds per square inch, the higher alkyl-homolog, 3-hexadecyl adipic acid, gave an increase of only 800 from 600 to 1400 pounds per square inch.

The dicarboxylic acids of this invention are useful

also for providing superior load carrying properties in lubricating oils which contain minor amounts of other agents which are non-reactive with the dicarboxylic acids, such as silicone anti-foaming agents, alkylphenol anti-oxidants, polyacrylate ester viscosity-index improvers, and the like.

We claim as our invention:

1. A lubricating oil composition comprising a major amount of lubricating oil and from about 0.1% to about 2% of an aliphatic dicarboxylic acid having the formula  $\text{HOOC}\text{C}_n\text{H}_{2n-m}\text{R}_m\text{COOH}$  wherein  $\text{R}$  in the side chain of the hydrocarbon group  $\text{C}_n\text{H}_{2n-m}\text{R}_m$  and is an alkyl radical of from 1 to 4 carbon atoms,  $n$  is an integer of from 3 to 6,  $m$  is an integer of from 1 to 6 inclusive and the total number of carbon atoms in all  $\text{R}$ 's is from 1 to 6.

2. The lubricating composition of claim 1 wherein the lubricating oil is a mineral lubricating oil.

3. The lubricating composition of claim 1 wherein the lubricating oil is selected from the group consisting of a polyoxy alkylene diol and the mono and diethers thereof.

4. The lubricating composition of claim 1 wherein the lubricating oil is an organic ester of an aliphatic dibasic acid.

5. A lubricating composition comprising a major amount of a mineral lubricating oil and from about 0.1% to about 2% of  $\text{C}_1\text{-C}_4$  alkyl substituted glutaric acid.

6. A lubricating composition comprising a major amount of a mineral lubricating oil and from about 0.1% to about 2% of a  $\text{C}_1\text{-C}_4$  alkyl substituted pimelic acid.

7. A lubricating composition comprising a major amount of a mineral lubricating oil and from about 0.1% to about 2% of a  $\text{C}_1\text{-C}_4$  alkyl substituted adipic acid.

8. A lubricating composition comprising a major amount of a mineral lubricating oil and from about 0.1% to about 2% of a  $\text{C}_1\text{-C}_4$  alkyl substituted suberic acid.

9. A lubricating composition comprising a major

amount of a mineral lubricating oil and from about 0.1% to about 2% of 3-methyl glutaric acid.

10. A lubricating composition comprising a major amount of a mineral lubricating oil and from about 0.1% to about 2% of 3,3-dimethyl glutaric acid.

11. A lubricating composition comprising a major amount of a mineral lubricating oil and from about 0.1% to about 2% of 3-methyl adipic acid.

12. A lubricating composition comprising a major amount of a mineral lubricating oil and from about 0.1% to about 2% of 2,3-dimethyl adipic acid.

13. A lubricating composition comprising a major amount of a mineral lubricating oil and from about 0.1% to about 2% of 2-methyl pimelic acid.

14. The lubricating composition of claim 9 containing a minor amount of a branched-chain alkanol.

15. The lubricating composition of claim 10 containing a minor amount of a branched-chain alkanol.

16. The lubricating composition of claim 11 containing a minor amount of a branched-chain alkanol.

17. The lubricating composition of claim 12 containing a minor amount of a branched-chain alkanol.

18. The lubricating composition of claim 13 containing therein a minor amount of a branched-chain alkanol.

25

References Cited in the file of this patent

UNITED STATES PATENTS

|              |                  |       |               |
|--------------|------------------|-------|---------------|
| 2,133,734    | Moser            | ----- | Oct. 18, 1938 |
| 2,158,096    | Werntz           | ----- | May 16, 1939  |
| 30 2,334,158 | Von Fuchs        | ----- | Nov. 9, 1943  |
| 2,402,825    | Lovell et al.    | ----- | June 25, 1946 |
| 2,452,319    | Patterson et al. | ----- | Oct. 26, 1948 |
| 35 2,452,320 | Kluge et al.     | ----- | Oct. 26, 1948 |
| 2,459,717    | Perry            | ----- | Jan. 18, 1949 |
| 2,548,493    | Robey            | ----- | Apr. 10, 1951 |
| 2,788,326    | Bondi et al.     | ----- | Apr. 9, 1957  |